

# United States Patent Office

2,873,214

Patented Feb. 10, 1959

1

2,873,214

## METHOD OF CHEMICALLY PLATING METALS

George L. Schnable, Lansdale, Pa., assignor to Philco Corporation, Philadelphia, Pa., a corporation of Pennsylvania

No Drawing. Application March 21, 1956

Serial No. 572,828

7 Claims. (Cl. 117—130)

The present invention relates to the chemical plating of metal coatings onto articles containing certain other base metals; and, more particularly, the invention relates to a novel method for chemically plating onto zinc, cadmium or manganese or alloys thereof, lower melting metal coatings which are more resistant to corrosion and are more readily soldered than the base metal.

In many industries today, particularly in the manufacture of electronic equipment, it is desirable to provide a metal coating on articles of zinc, cadmium, manganese or alloys of two or more of these, which is more resistant to corrosion, more readily soldered and melts at a lower temperature than the base metal. Attempts to do this by immersing the base metal into a molten bath of the coating metal covered by a suitable flux results in coatings the thickness of which cannot be controlled. Moreover, the high surface tension of certain of metals in molten form, most notably indium, makes wetting of irregular surfaces on the base metal difficult. Certain of the lower melting metals can also be electroplated out of aqueous solutions onto the base metal. However, in this case the deposits are crystalline, and have a relatively large surface area. Even with plating solutions having good "throwing power" irregular objects are unevenly coated. In order to obtain smooth coatings, the electroplated object must subsequently be immersed in a hot flux to melt the deposit. Of course, when the base metal article is very fine or complex, the making of the necessary electrical contacts for electroplating is difficult rendering electroplating impractical. Attempts to chemically plate the lower melting metals onto the base metal out of aqueous solution have failed inasmuch as the deposit is spongy and otherwise unsatisfactory, and deposition in such a system stops as soon as an initial layer of deposit is formed unless an extraneous reducing agent is added to the solution.

It is the principal object of the present invention to provide a novel method for providing metal coatings on articles containing zinc, cadmium, manganese or alloys of two or more of these.

Another object of the present invention is to provide a novel method for providing, by a chemical plating operation, smooth, uniform coatings, on zinc, cadmium, manganese or alloys of two or more of these, comprising metal which is more corrosion-resistant and more easily soldered than the base.

Still another object of the present invention is to provide a novel method for forming, by chemical plating, smooth, dense, homogeneous and uniform metal coatings of the type mentioned above on bases of zinc, cadmium, manganese or alloys of two or more of these even when the base metal presents a highly irregular or complex surface.

Other objects will become apparent from a consideration of the following specification and the claims.

The method of the present invention comprises immersing the article to be coated comprising at least one of the metals selected from the group consisting of zinc, cadmium and manganese in a liquid, non-aqueous bath comprising salt of metal other than the base metal selected and more noble than the base metal, until the desired amount of more noble metal is chemically plated on the article in a coating, said bath being at a temperature below

2

the solidus point of the base metal but above the liquidus point of the metal coating.

It has been found that simple immersion of zinc, cadmium or manganese, or alloys of two or more of these, in a hot, non-aqueous bath comprising salt of metal, other than the particular base metal selected and more noble than the particular base metal, especially those selected from the group consisting of bismuth, indium, tin, lead, thallium, cadmium and zinc, at a temperature below the solidus point of the base metal results in chemical plating of the more noble, lower-melting metal onto the base in the form of a molten coating, when the temperature of the bath is above the liquidus point of the metal coating. In this way a coating of any desired thickness can be formed. Upon removal of the coated article from the bath, the molten metal rapidly solidifies to provide a uniform coating of any desired thickness which is dense, smooth and homogeneous. Moreover, in addition to the high quality of the coating, the coating is uniform over irregular surfaces and even on inside, but exposed, surfaces.

The present process, being a chemical plating procedure based on the phenomenon of simple chemical displacement due to relative differences in position in the electromotive series, does not rely on any flow of current, as in electroplating, nor on an extraneous reducing agent. There is no need to maintain electrical contact as in the case of electroplating so that the fineness or complexity of the parts is not material.

30 The present method is applicable to the coating of articles comprising at least one of the metals selected from the group consisting of zinc, cadmium and manganese, that is zinc, cadmium or manganese or alloys containing two or more of these. In such alloys the composition may vary widely from those containing substantial amounts of each metal to those in which one of the constituents is present in only a minute amount, such as about 0.1%, by weight. Examples of such alloys are cadmium-zinc alloys containing between about 0.1—99.9% cadmium to 99.9—0.1% zinc, by weight, the eutectic being 17% zinc to 83% cadmium.

Such base metals are readily wetted by the molten metal, and the molten metal deposit adheres readily thereto. Any desired amount of metal can be deposited, 45 from a very thin molecular film to heavy deposits depending upon the results desired, the nature of the base and the amount of plating metal in the bath. In fact if the bath contains an amount of plating metal at least chemically equivalent to the base metal, the base metal can be completely displaced by the more noble metal. Thus plating can be continued until all of the base metal has been so displaced, or, the procedure can be stopped short of complete displacement to provide a coating of any desired thickness. The complete displacement of base 50 metal is a practical consideration in many instances. For example, where it is desired to apply a small dot of indium to a germanium base, indium being soft and difficult to handle as small pellets, a dot of zinc or the like may be applied to the base and the zinc then displaced by indium in accordance with the present procedure.

The base metal is soluble in the plated metal forming, as the metal coating, an alloy in molten form therewith. It is this feature that permits plating to continue once a coating is formed since the formation of the alloy makes base metal available at the interface between the coating and the bath. The exact composition of the alloy formed may vary widely depending upon the phase diagram of the system and the temperature of operation, the higher the temperature, the more soluble the base metal in the coating. The concentration of base metal in the coating may go as low as about 0.01 atomic percent.

The metal plated out must be more noble than the base metal onto which it is deposited. Examples of metals that may be deposited on zinc, cadmium or manganese or alloys thereof in accordance with the present procedure are bismuth, indium, tin, thallium and lead. In accordance with the present procedure, zinc may also be deposited on manganese, cadmium may be deposited on manganese and cadmium may be deposited on zinc. Combinations of metals may be deposited by use of salts of two or more of the stated metals in the bath. As mentioned above, in any case the coating is actually an alloy, one constituent of which is the base metal and the other or others of which is the more noble metal or metals from the bath.

As stated, the procedure comprises simply immersing the base metal into a liquid, non-aqueous bath comprising salt of more noble metal to be deposited at a temperature below the solidus point of the base metal but above the liquidus point of the metal coating formed. The metal to be deposited will exist, just prior to deposition, in solution in the bath in the form of ions. The bath may be a molten salt bath comprising molten salt of metal to be deposited or may be a solution of salt of metal to be deposited in a high boiling organic solvent therefor. In the case of the fused salt bath, the bath may consist substantially entirely of molten salt of the more noble metal. For example, a salt of indium, lead, thallium, bismuth or tin, or of cadmium when cadmium is to be deposited on manganese or zinc or of zinc when zinc is to be deposited on manganese, which has a melting point below the solidus point of the base metal selected, may be simply melted to form the bath. Of such salts the halides are especially suitable, particularly the chlorides and bromides. Examples of suitable salts, in this connection, are indium monochloride, stannous chloride, thallous chloride, plumbous bromide, bismuth chloride, cadmium chloride, zinc chloride, and the like. It is preferred that the more noble metal be in a lower valent state in the bath. For example, preferably indium exists in the bath at a valence below three, that is, one and/or two, tin exists as stannous ions, lead as plumbous ions and thallium as thallous ions. The maintenance of the multivalent metals in a lower valent state will present no problems to those skilled in the art, and any one of several expedients serving to maintain the metal in a reduced ionic state may be employed. For example, the surface of the bath may be covered with a non-oxidizing, that is a neutral or reducing, atmosphere, such as carbon dioxide, hydrogen, helium, argon, nitrogen, or the like. The multi-valent metal ions may also be prevented from oxidizing to the highest valent state by maintaining, in the bath, a body of the elemental metal as such.

In addition to salt of more noble metal, the fused salt bath may contain other salts. When the bath contains salts of metals it is not desired to deposit, the metals will, as a general rule, not be more noble than the base metal. For example, in the case of plating onto a base comprising zinc or cadmium, salt of the metal to be deposited may be mixed with a zinc salt, the zinc salt merely serving as diluent or solvent. The above-stated general rule is subject to some exception where the metal of the diluent salt and the more noble metal are relatively far apart in the electromotive series in which case the most noble metal in solution will selectively plate out on the base even though the metal of the diluent salt is somewhat more noble than the base metal. For example, in depositing indium on manganese, the bath may also contain a zinc salt in which the indium alone will be deposited. Salts of the alkali metals, such as their halides, may be employed as diluents or solvents. Non-metal salts, such as ammonium salts, may also be employed. Examples of fused salt mixtures serving merely as diluent or solvent are a combination of zinc chloride and ammonium chloride, especially in a 3 to 1 weight

ratio (the eutectic melting at 180° C.); a mixture of lithium chloride and potassium chloride, especially in a 5 to 6 weight ratio (the eutectic melting at 352° C.); and the like.

5 The use of a diluent salt is advantageous in many instances to control the rate of deposition. The rate of chemical plating appears to be directly proportional to the concentration of ions of metal to be deposited. For example, zinc immersed in molten stannous chloride at 300° C. reacts vigorously with heat evolution to form molten tin-zinc alloy. When, however, zinc metal is immersed in a molten mixture containing equal parts, by weight, of zinc chloride and stannous chloride, the reaction proceeds smoothly, coating the zinc with molten tin-zinc alloy at the rate of about 0.08 inch per minute.

10 On the other hand, the bath may comprise a solution of salt of the more noble metal in a high boiling organic compound, or mixture of such compounds, which at the temperature of operation serves as a solvent for the salt and in which ionic conduction occurs at the temperature of operation. Such compounds are normally polar and will have a boiling point above the temperature of operation. Examples of polar organic compounds that may be employed are the polyhydric alcohols, such as glycerols, 20 the glycols, for instance ethylene glycol, the polyethylene glycols, especially diethylene glycol, 1,2,4-butane triol, sorbitol, and the like; glycol derivatives, such as ethylene glycol monobutyl ether, and the like; high boiling amines, such as triethanolamine, N,N,N',N'-tetrakis (2-hydroxy-propyl) ethylene diamine, and the like; amides such as acetamide; phenol; phthalic anhydride; benzoic acid; and the like. The organic material may be solid at ordinary temperatures so long as it is liquid at the temperature of operation, as is the case with many of those materials mentioned above.

25 The concentration of the metal, in ionic form, in the bath is relatively immaterial since the process is selective and quantitative. In other words, when only small amounts of metal are to be plated on a small article, a concentration of the plating metal as little as about 0.001 normal, at the temperature of operation, may be sufficient. On the other hand, when the bath is made up entirely of salt of the plating metal, the metal, in 30 ionic form, will make up 100 atomic percent of the cations of the bath. Advantageously, the concentration of plating metal in the bath is at least about 0.01 normal at the temperature of operation.

35 During operation, the bath will be at a temperature below the solidus point of the base metal, preferably at 40 least 40° C. below, but above the liquidus point of the metal coating. Hence, the exact temperature of the bath will depend upon the system employed and particularly upon the metal coating formed. Since the metal coating formed is an alloy, the temperature of the bath will be 45 above the liquidus point of that alloy although it may well be below the melting points of each of the individual metals. For example, when tin is chemically plated onto cadmium in accordance with the present process there is formed a tin-cadmium alloy which melts below 200° C. Although cadmium itself melts at 321° C. and tin itself melts at 232° C., the bath in this case may be operated at a temperature in the neighborhood of about 200° C. to form the molten alloy. Likewise, when lead is 50 chemically plated onto cadmium in accordance with the present procedure, there is formed a lead-cadmium alloy which melts below 280° C. The bath in such case can be operated at a temperature of about 280° C., although the melting point of cadmium is 321° C. and the melting point of lead is 327° C.

55 Once the base metal article is immersed in the bath at operating temperature molten metal begins to form thereon. The base metal article is left in the bath until the desired amount of coating has been so formed. Then the coated article is removed from the bath and the molten metal is permitted to solidify. The coated article

may then be subjected to cleaning and finishing operations, as desired, such as rinsing, etching, and the like.

Agitation is advantageous during the procedure since it helps to provide a reproducible rate of chemical plating as local heating of the immersed metal due to heat evolved during the reaction is avoided. Agitation also assures that the concentration of ions in the vicinity of the immersed metal does not change as the reaction proceeds.

The process of the present invention will be more readily understood from a consideration of the following specific examples which are given for the purpose of illustration only and are not intended to limit the scope of the invention in any way.

*Example I*

A saturated (at 25° C.) solution of indium trichloride in ethylene glycol is heated to 180° C. Pieces of zinc metal immersed in this solution at 180° C. are soon covered with a smooth, uniform coating of molten indium metal containing a small amount of zinc. Upon the removal of the coated zinc metal from the bath, the coating rapidly solidifies, and the assembly is washed with plain water to remove any adhering plating bath.

*Example II*

A saturated (at 25° C.) solution of indium trichloride in glycerol is heated to 180° C. Pieces of zinc metal immersed in this bath as in Example I are quickly plated with a smooth, uniform coating of molten indium metal containing a small amount of zinc which solidifies upon removal of the coated object from the bath.

*Example III*

Stannous chloride is melted and maintained at a temperature of 300° C. Pieces of zinc metal immersed in the molten stannous chloride at this temperature rapidly become covered with a smooth, uniform coating of molten tin containing a small amount of zinc. Upon the removal of the coated zinc objects from the bath, the coating solidifies and the assemblies are washed with water.

*Example IV*

A mixture of ten grams of zinc chloride and ten grams of stannous chloride are maintained at a temperature of 300° C. Pieces of zinc metal immersed in this bath are coated with molten tin containing a small amount of zinc, but at a substantially slower rate, about 80 mils per minute, than is the case with Example III.

*Example V*

Stannous chloride is melted and maintained at a temperature of 300° C. Cadmium metal immersed in the molten stannous chloride is rapidly covered with a smooth, uniform coating of molten tin containing a small amount of cadmium at an estimated plating rate of about 30 mils per minute.

*Example VI*

One gram of indium trichloride is added to 10 grams of glycerol and the solution heated at 180° C. Cadmium immersed in this bath is provided with a smooth, uniform coating of molten indium containing a small amount of cadmium at an estimated plating rate of about 5 mils per minute.

*Example VII*

One gram of stannous chloride is added to 10 grams of glycerol and the solution heated at 200° C. Cadmium immersed in this bath is provided with a molten coating of cadmium-tin alloy.

*Example VIII*

One gram of plumbous bromide is added to 10 grams of a zinc chloride-ammonium chloride eutectic (3 to 1, by weight, melting point 180° C.) and heated at 280° C. Cadmium immersed in this bath is provided with a smooth, uniform coating of cadmium-lead alloy.

*Example IX*

One gram of indium trichloride is added to 10 grams of glycerol and the solution heated to 220° C. Manganese immersed in this bath is provided with a smooth, uniform coating of molten indium containing a small amount of manganese at an estimated plating rate of about 0.5 mil per minute.

*Example X*

One gram of indium trichloride is added to 10 grams of a molten lithium chloride-potassium chloride eutectic (5:6, by weight, melting point 352° C.) and the solution heated at a temperature of 420° C. Manganese immersed in this bath is provided with a smooth, uniform coating of indium containing a small amount of manganese at an estimated plating rate of about 1 mil per minute.

*Example XI*

One gram of cadmium chloride is added to 10 grams of zinc chloride and the mixture heated at 350° C. Zinc immersed in this bath is coated with molten cadmium containing a small amount of zinc.

Considerable modification is possible in the selection of the combination of base metal and plating metal and the other constituents of the bath as well as in the exact techniques followed without departing from the scope of the invention.

I claim:

1. The method of coating articles comprising at least one of the metals selected from the group consisting of zinc, cadmium and manganese with a lower melting metal which comprises immersing said article in a solution of salt of metal other than the selected base metal and more noble than the selected base metal in a polar organic compound until the desired amount of more noble metal is deposited on the article in a coating through displacement of base metal in the form of an alloy with said base metal, said solution being at a temperature below the solidus point of the base metal but above the liquidus point of the metal coating.
2. The method of claim 1 wherein the organic compound is a polyhydric alcohol.
3. The method of displacing a base metal comprising at least one of the metals selected from the group consisting of zinc, cadmium and manganese with a lower melting metal which comprises immersing said base metal in a liquid, non-aqueous bath comprising salt of metal other than the selected base metal and more noble than the selected base metal until at least a portion of said base metal has been displaced by said more noble metal forming an alloy therewith in molten form, said bath being at a temperature below the solidus point of the base metal and below the solidus point of said more noble metal but above the liquidus point of said alloy.
4. The method of claim 3 wherein substantially all of said base metal is displaced.
5. The method of claim 3 wherein said liquid non-aqueous bath is a molten salt bath.
6. The method of claim 5 wherein said molten salt bath comprises, in addition to salt of the said more noble metal, other salt selected from the group consisting of ammonium salts and salts of metals no more noble than the selected base metal.
7. The method of claim 5 wherein the molten salt bath consists essentially of salt of the said more noble metal.

References Cited in the file of this patent

UNITED STATES PATENTS

70 2,667,433 Gebhardt \_\_\_\_\_ Jan. 26, 1954

OTHER REFERENCES

75 Hoge: Protective Metallic Coatings From Molten Salts, Metal Progress, November 1947, vol. 52, pages 819-823.